

# UNITED STATES PATENT OFFICE.

LORENZ KLÖPFER, OF MUNICH, GERMANY.

## COLORING AND BRONZING LEATHER.

SPECIFICATION forming part of Letters Patent No. 295,653, dated March 25, 1884.

Application filed September 4, 1883. (No specimens.)

*To all whom it may concern:*

Be it known that I, LORENZ KLÖPFER, a subject of the Emperor of Germany, and residing at Munich, Germany, have invented new and useful Improvements in Treating Leather for Ornamental Purposes, of which the following is a specification.

This invention relates to the production of embossed, colored, or gilded leather or similar materials, and to the coating of the same with metal.

The various methods or processes heretofore employed for embossing leather have not given satisfactory results, because the leather, being pressed by engraved steel rollers heated by steam, loses its original flexibility, and is consequently useless for upholstering purposes. On leather thus prepared, whether coated with metal or having its natural surface, colors cannot be durably applied.

The present invention, besides obviating the above defects, offers many advantages.

In carrying out my invention I proceed as follows: The leather to be pressed is wrapped in a piece of cloth moistened with boiled water to which a small quantity of milk has been added. The leather remains in this cloth for from six to ten hours, according to the quality or kind of leather—such as roan, morocco, calf, or the like—and this time is also dependent upon the color, gilding, or metal covering which it is intended to apply upon the leather, &c. The pressing or embossing which follows the preliminary working is effected without heat by means of stones or metal plates. However, I prefer to use lithographic stones on which the desired pattern is etched or engraved. Patterns thus produced have remarkable advantages, namely: When the plate is pressed upon the leather, the latter, whether natural or colored, receives a uniform ground color or tone. Another advantage is that special colors—such as ultramarine—can be pressed upon the leather which is gilt or covered with a metallic coating. The pressing or embossing is performed in the ordinary press. The leather or similar material, having been treated as above described, is then thoroughly dried, and after six or eight days is washed with a sponge dipped in a mixture of five parts of whites of eggs, two parts of glycerine, and one part of distilled water. By this treatment the

leather acquires a permanent flexibility and a greater durability than when prepared by other processes, and is also more suitable for industrial purposes, especially where soft and elastic leather is required.

In order to gild, silver, or color the leather or similar material with a metal coating in such a manner that it shall not be affected by the above-described treatment, the said leather is covered, according to its quality and mode of preparation, whether roan, morocco, or calf, with a solution of shellac and then dried, after which the said leather is covered with a mixture of one-half pound of crude collodion and thirty drops of castor-oil, this mixture being diluted with alcohol and sulphuric ether mixed in the proportion of two parts of alcohol with one of sulphuric ether. This operation is repeated one or more times, according to the number of fatty cells existing in the leather.

A very thin layer of size or other suitable mixture is placed upon the leather, and is allowed to become almost dry, and while the same is still adhesive the gold-leaf or other metal leaf is then laid upon the same, when the leather may be embossed, as above described.

The leather prepared according to the above-described process remains thoroughly flexible and soft, and its gilding is very durable, and the leather is applicable for all embossing processes, whatever the pattern may be.

Having thus described my invention, what I claim as new, and desire to secure by Letters Patent, is—

1. The process of treating leather preparatory to coating with metal and embossing it, consisting of first wrapping the leather in a cloth moistened with a solution of water and milk, drying it, then washing it with a mixture of white of egg, glycerine, and water, and then covering the leather first with a varnish and then with a flexible collodion compound, and finally applying a thin coating of size or other similar mixture, and applying the metal coating before the mixture has become dry, substantially as set forth.

2. In the process of treating leather preparatory to coating with metal and embossing it, the method of rendering the leather pliable and soft, consisting in wrapping the leather in a cloth moistened with boiled water and milk,

then drying it, and then washing the leather with a mixture of white of egg, glycerine, and distilled water, substantially as set forth.

3. In the process of treating leather preparatory to coating with metal and embossing it, the method of forming a good adhesive surface for the reception of the metal, consisting in thoroughly drying the leather, previously rendered pliable, applying a solution of shellac, and coating the leather with a mixture of crude collodion, castor-oil, alcohol, and sulphuric

ether, applying a thin coating of size or similar mixture, on which the desired color or leaf is laid, substantially as set forth.

In testimony whereof I have signed my name 15 to this specification in the presence of two subscribing witnesses.

LORENZ KLÖPFER.

Witnesses:

T. MERZ,  
EMIL HENZEL.